

## UNITED STATES PATENT OFFICE.

HAROLD H. OSBORNE, OF CLEVELAND, OHIO, ASSIGNOR TO AMERICAN MAGNESIUM CORPORATION, OF NIAGARA FALLS, NEW YORK, A CORPORATION OF NEW YORK.

## CASTING FREELY OXIDIZABLE METAL.

No Drawing.

Application filed March 6, 1922. Serial No. 541,569.

*To all whom it may concern:*

Be it known that HAROLD H. OSBORNE, a citizen of the United States, residing at Cleveland, in the county of Cuyahoga and State of Ohio, has invented certain new and useful Improvements in Casting Freely Oxidizable Metals, of which the following is a specification.

My invention relates to the casting of magnesium and high magnesium alloys and other freely oxidizable metals and has for its object to provide a binder for "green sand" molds; i. e., non-baked, which will not oxidize the molten metal when it comes in contact therewith. The ordinary binding material for green sand molds contains water, but this cannot be used in casting magnesium and similar metals due to the fact that the metal will oxidize when it comes in contact with the water. This has accordingly necessitated the selection of a non-aqueous binder for such molds.

To be commercial, sand prepared with such a binder must lift in the flasks, part readily from itself and the pattern, shake freely from the casting, leave the casting with a clean metallic surface and generally produce sound castings in the usual sense. In the repeated use of the binding liquid it must not develop gumming fatty acids under the action of the hot metal but must volatilize or form gases only.

In selecting such a binder, consideration must also be given to its molding qualities. In the use heretofore of other non-aqueous binders, such as heavy lubricating oils, the binding qualities depend largely upon the viscosity and adhesiveness of the binder itself. While the use of such a binder prevents burning of the metal, difficulty is experienced in making the sand stick in the foundry flask and in maintaining the shape of the mold.

I have discovered that glycerine not only prevents oxidation of the metal but also has desirable molding qualities. It mixes with the sand very readily and its binding action seems to come from the wetting of the clay in the sand, thus making available the natural binding properties of the clay, as in the case of water bound sand. Glycerine bound sand looks and feels very much like water bound sand and in its molding action behaves very similar to water sand.

One method of mixing and using glycerine sand is as follows: The sand is heated until thoroughly dried and then while still warm, it is mixed with anhydrous or nearly anhydrous glycerine, preferably dynamite glycerine, in the proportions of about one pint of glycerine to fifteen or twenty pounds of dry sand. The proportion of glycerine and sand will of course vary with different grades of sand. After the glycerine and sand have been completely and thoroughly mixed, the mixture is allowed to soak for several hours, preferably over night, and it is then ready for use. From this point on, it is molded and handled exactly as is water bound sand, except that after the castings are shaken out, the sand is merely cut over and mixed and is then ready for subsequent use again. Glycerine or glycerine rich sand is added to the used sand, only over relatively long intervals as the consistency of the sand demands and to make up for the slight loss of binder through volatilization and decomposition, when the hot metal is poured into the mold.

Some of the advantages of a glycerine binder may be enumerated as follows:

It prevents the oxidation of the easily oxidized metals, which takes place when these metals are cast into water bound molds. It makes possible the casting of these metals into "green" molds, i. e. not baked, thus effecting a great saving in time, fuel, labor and molding equipment. Its similarity to water and dissimilarity to oil in the manner in which it wets the clay of the sand, gives the sand the properties by virtue of which it can be formed into a mold which has all the properties that a mold should have in order to give satisfactory castings, i. e., sufficient strength to "stand up" and porosity to permit the venting of trapped or liberated gases. It has permanency, in that after the sand has been mixed with the glycerine binder, there is very little deterioration, except for the necessity of the occasional addition of glycerine or glycerine rich sand to replace the glycerine which has been lost through volatilization and decomposition and perhaps for the necessity, at long intervals, of heating the sand for a while at a moderate temperature to drive off any moisture which the glycerine may have absorbed from the atmosphere because of its hygro-

scopic nature. It chills the metal quickly and volatilizes cleanly in the mold leaving a dry layer of sand therein.

Glycerine is a trihydric alcohol having the formula  $C_3H_5(OH)_3$ . It is a thick colorless syrup at ordinary temperatures, boils at 290 degrees C. and is miscible with water and alcohol in all proportions. Other polyhydric alcohols are closely related in physical and chemical properties to glycerine and accordingly may be used as equivalents therefor where their price would permit.

In referring herein to anhydrous glycerine, it will be understood that on account of the hygroscopic character of the compound, it will not always remain absolutely water free; but the small amount of water which it absorbs in this manner does not, however, materially affect its use.

It will be understood therefore that although glycerine is the preferred binding agent, I do not intend to so limit myself, but comprehend within the discovery those substances having similar properties to those of glycerine, and properly falling within the scope and spirit of the appended claims.

I claim:

- 30 1. A sand mold having a binder containing glycerine.
2. A green sand mold having a binder of substantially anhydrous glycerine.
3. A green sand mold having a binder containing a polyhydric alcohol.
- 35 4. The process of making a casting of freely oxidizable metal, comprising forming a mold from sand rendered moldable by being mixed with a glycerine containing binder and casting said metal in said mold.
- 40 5. The process of making a magnesium or high magnesium alloy casting comprising forming a mold from sand freed from water and rendered moldable by being mixed with glycerine and casting said metal in said mold.
- 45 6. The process of making a casting of

magnesium and high magnesium alloys which comprises forming a mold from sand with a binder containing glycerine and casting the molten metal in the said mold.

7. The method of making molds comprising mixing with a clay-containing sand a substantially anhydrous liquid binder which increases the molding qualities of the sand by acting on the clay containing portions to develop its plasticity.

8. The method of making a casting of magnesium and high magnesium alloys which comprises forming a mold from sand with a substantially anhydrous liquid binder which increases the molding qualities of the sand by acting on the clay containing portions to develop its plasticity, and casting molten metal in the said mold, the said binder being volatilizable at the temperature of the molten metal.

9. The process of making a magnesium or high magnesium alloy casting which comprises pouring the molten metal into a sand mold having a substantially non-aqueous binder which on being heated by the molten metal will give off gases which protect the magnesium from oxidation.

10. The process of casting freely oxidizable metals which comprises pouring the molten metal into a mold containing a substance which on being heated by the molten metal will give off gases which protect the metal from oxidation.

11. The process of casting magnesium and high magnesium alloys in sand molds comprising mixing with the sand a substance which on being heated by the molten metal will give off gases which protect the magnesium from oxidation.

In testimony whereof I affix my signature.

HAROLD H. OSBORNE.

Witnesses:

O. WILHELMY,  
W. HOLZHAUER.